

## UNITED STATES PATENT OFFICE

2,525,502

PRODUCTION OF PHENAZONIUM  
DYESTUFF IMAGES

Vsevolod Tulagin, Phillipsburg, N. J., and Willy A. Schmidt, Easton, Pa., assignors to General Aniline & Film Corporation, New York, N. Y., a corporation of Delaware

No Drawing. Application December 23, 1947,  
Serial No. 793,534

7 Claims. (Cl. 95—6)

1

The present invention relates to the production of blue-green or cyan phenazonium dyestuff images by color development of an exposed silver halide emulsion with an ortho-phenylenediamine type developer in the presence of a 7,8-benzoquinoline as the color former.

Schmidt and Tulagin copending application Serial Number 640,382, filed January 10, 1946, now Patent No. 2,486,440, describes the production of phenazonium dyestuff images by color developing an exposed silver halide emulsion with a color developer comprising an ortho-phenylenediamine type developer in the presence of various color formers. Among the color formers mentioned are those containing a phenolic hydroxyl group which couples in para position to such group. It has been observed that with the color formers mentioned in said copending application, the most common color of the dyestuff images obtained is either red or that shade of red known in the photographic art as magenta. As a matter of fact, it may be said that these are the only shades which are obtainable from phenols or naphthols when the coupling reaction takes place para to the phenolic hydroxyl group. This limitation on the shades of the dyestuffs produced according to the method of said application imposes a restriction on its use in three-color photography.

It has now been discovered that cyan or blue-green phenazonium dyestuff images are obtained by color developing an exposed silver halide emulsion with an ortho-phenylenediamine type developer in the presence of a benzoquinoline containing in the hetero ring thereof an auxochromic group such as hydroxyl, amino, or substituted amino.

The production of phenazonium dyestuff images by the utilization of such color formers and silver halide emulsions and color developers containing such color formers constitute the purposes and objects of the present invention.

The benzoquinolines contemplated for employment herein may be represented by the following structural formula:

2



15 wherein R is an auxochromic group, such as hydroxy, amino, arylamino, i. e., phenylamino, anisylamino, arsonophenylamino, sulfophenylamino, sulfoacetylaminophenylamino; alkylamino, i. e., methylamino, ethylamino, propylamino, decylamino, laurylamino, tetradecylamino, stearylamino, and the like; or aryl-alkylamino, i. e., methyl-phenylamino, and the like; R1 is hydrogen or a lower alkyl such as methyl, ethyl, propyl, butyl, and the like; and the OH group indicated is in the  $\beta$ -position of the naphthalene ring system.

20 Examples of compounds embraced by these formulas and which have been found to be suitable for producing the desired cyan dye images are the following:

1.



30

2-methyl-4,5'-dihydroxy-7,8-benzoquinoline

2.



40

2-methyl-4,4'-dihydroxy-7,8-benzoquinoline



The benzoquinolines employed as color formers in this invention can be prepared by the following general methods: Thus, compounds 1, 2, 4 and 5 can be prepared by reacting the appropriate aminonaphthol with ethyl acetoacetate in the presence of a trace of hydrochloric acid and then heating the intermediate reaction product in mineral oil to produce the benzoquinoline. Compound 3 is obtained by reacting 1-amino-7-naphthol with diketene and then heating at 85° C. the reaction product in sulfuric acid. Compounds 6, 7, 8, 11 and 12 can be prepared by reacting compound 2 with a mixture of ethyl bromide and sodium hydroxide, treating the compound obtained with phosphorus oxychloride, followed by reaction with a mixture of hydrobromic and acetic acids to obtain 2-methyl-4-chloro-4'-hydroxy-7,8-benzoquinoline. Upon heating of the latter compound in the presence of a trace of hydrochloric acid with p-aminophenylarsonic acid, ammonia, sulfanilic acid, aniline and lauryl amine respectively, the desired compounds are

obtained. Compounds 9 and 10 can be obtained by reacting 2-methyl-4-chloro-4'-hydroxy-7,8-benzoquinoline with p-phenylenediamine and monotetradecyl-p-phenylene diamine and then reacting the resultant compounds with a mixture of chloroacetyl chloride and acetic acid and finally heating with an aqueous solution of sodium sulfite.

The color formers are employed either in the emulsion or in the developer. However, where they contain a group preventing diffusion, they are preferably used in the emulsion. Examples of compounds falling within such category are compounds 8 and 11 above.

The color developers which are employed are, as stated, of the ortho-phenylenediamine type, a number of examples of which are referred to in the aforesaid Schmidt and Tulagin application. Suitable developers of this class are:

4,6-dianilino metanilic acid  
4,6-bis-(p-methoxy-phenylamino)-metanilic acid  
4-(o-methoxy-phenylamino)-6-(p-methoxy-phenylamino)-metanilic acid  
4,6-bis-(o-methoxy phenylamino)-metanilic acid  
4-(p-sulfo-phenylamino)-6-dimethylamino metanilic acid, and the like.

The invention may be effectuated so as to use the color developing method for producing colored negatives, colored positives, or reversed images. These general methods are conventional in the art, being dependent for their efficacy upon the point at which color development takes place.

The invention is further illustrated by the following examples, but it is to be understood that the invention is not restricted thereto.

*Example 1*

To 1 kilo of a silver bromide iodide emulsion is added .7 gram of 2-methyl-4-(4"-N-tetradecylsulfoacetamido-aniline)-4'-hydroxy-7,8-benzoquinoline, and the mixture is coated on a suitable support. The resulting film is exposed and developed in a black and white developer. The film is thoroughly washed and the residual silver halide re-exposed and developed in a developer of the following composition:

|                              |                   |      |
|------------------------------|-------------------|------|
| 4,6-dianilino metanilic acid | grams             | 1.5  |
| Sodium sulfite               | do                | 60   |
| Potassium carbonate          | do                | 40   |
| Pyridine                     | cubic centimeters | 12   |
| Water                        | do                | 1000 |

The film is washed, bleached and fixed in the conventional manner to yield cyan phenazonium dyestuff images of high contrast.

*Example 2*

A silver bromide emulsion is exposed and color developed in a developer of the following constitution:

|                                            |                   |      |
|--------------------------------------------|-------------------|------|
| 4,6-dianilino metanilic acid               | grams             | 1.5  |
| Sodium sulfite                             | do                | 60   |
| Potassium carbonate                        | do                | 40   |
| Pyridine                                   | cubic centimeters | 12   |
| 2-methyl-4,5'-dihydroxy-7,8-benzoquinoline | grams             | 1    |
| Water                                      | cubic centimeters | 1000 |

The film is washed, bleached and fixed in the customary manner. A negative cyan phenazonium dyestuff image remains.

The following table illustrates the color of the dyestuff images obtained when using other color formers with the developer of Example 1:

6  
Table 1

|    | Coupler                                                            | Color of Formed Dye |
|----|--------------------------------------------------------------------|---------------------|
| 5  | 2-methyl-4,4'-dihydroxy-7,8-benzoquinoline                         | Greenish blue.      |
|    | 2,4'-dihydroxy-4-methyl-7,8-benzoquinoline                         | Do.                 |
|    | 2-methyl-4(4"-arsonoanilino)-4'-hydroxy-7,8-benzoquinoline         | Do.                 |
|    | 2-methyl-4(4"-sulfoanilino)-4'-hydroxy-7,8-benzoquinoline          | Do.                 |
| 10 | 2-methyl-4(4"-sulfoacetamidoaniline)-4'-hydroxy-7,8-benzoquinoline | Do.                 |

Various modifications of the invention will occur to persons skilled in the art, and we therefore do not intend to be limited in the patent granted except as necessitated by the prior art and the appended claims.

We claim:

1. The process of producing cyan phenazonium dyestuff images by color forming development which comprises exposing a silver halide emulsion and developing the same with an ortho-phenylenediamine type developer in the presence of a color former selected from the group having the following formulas:



30 and



35 wherein R is an auxochromic group selected from the class consisting of hydroxy and amino groups, R1 is lower alkyl, the OH indicated in the formula is in the beta-position of the designated benzo ring and R and R1 are both in the heterocyclic ring.

40 2. The process as defined in claim 1, wherein the color former is 2-methyl-4,5'-dihydroxy-7,8-benzoquinoline.

45 3. The process as defined in claim 1, wherein the color former is 2-methyl-4-(4"-tetradecylsulfoacetamidoaniline)-4'-hydroxy-7,8-benzoquinoline.

50 4. A photographic silver halide emulsion containing as a color former capable of yielding cyan phenazonium dyestuff images when color developed with an ortho-phenylenediamine type developer a compound selected from the group having the following formulas:



55 and



wherein R is an auxochromic group selected from the class consisting of hydroxy and amino groups, R<sub>1</sub> is lower alkyl, the OH indicated in the formula is in the  $\beta$ -position of the designated benzo ring and R and R<sub>1</sub> are both in the heterocyclic ring.

5. A photographic developer containing as the reducing agent a 4,6-diamino metanilic acid and as the color former a compound selected from the group having the following formulas:



and



where R is an auxochromic group selected from the class consisting of hydroxy and amino groups, R<sub>1</sub> is lower alkyl, the OH indicated in the formula is in the  $\beta$ -position of the designated benzo ring and R and R<sub>1</sub> are both in the heterocyclic ring, said compound being free from groups rendering said compound non-diffusing in photographic emulsions.

5 10 6. The photographic developer of claim 5 wherein the color former is 2-methyl-4,5'-dihydroxy-7,8-benzoquinoline.

7. The photographic silver halide emulsion defined in claim 4 wherein the color former is 2-methyl-4-(4''-N - tetradecyl-sulfoacetamidoaniline)-4'-hydroxy-7,8-benzoquinoline.

VSEVOLOD TULAGIN.  
WILLY A. SCHMIDT.

#### REFERENCES CITED

20 The following references are of record in the file of this patent:

#### UNITED STATES PATENTS

| Number       | Name            | Date         |
|--------------|-----------------|--------------|
| 25 2,313,138 | Frohlich et al. | Mar. 9, 1943 |